

2,962,356

## CORROSION INHIBITION

Iral B. Johns, Dayton, Ohio, assignor to Monsanto Chemical Company, St. Louis, Mo., a corporation of Delaware

No Drawing. Filed Sept. 9, 1953, Ser. No. 379,283

5 Claims. (Cl. 23—139)

This invention relates generally to the inhibition of corrosion of metallic titanium. In its more specific aspects it relates to the inhibition of acid attack upon metallic titanium. A particularly useful embodiment of the present invention involves the inhibition of corrosion by aqueous acid solutions containing inorganic salts dissolved therein.

Metallic titanium is becoming an increasingly important material of construction, particularly because of its high strength to weight ratio and its resistance to certain types of corrosion, such as corrosion by sea-water or other salt solutions. One of the disadvantages of the metal is, however, that it is subject to acid attack, particularly by strong acids, such as the mineral acids, e.g., hydrochloric and sulfuric acids. It is, therefore, a general object of the present invention to provide a novel method of inhibiting the attack by acids upon metallic titanium.

While the inhibition of acid attack upon metallic titanium is obviously very useful in situations involving titanium equipment which is handling acids or acidic solutions, there is another and possibly more important utility for the present invention in connection with various processes for producing metallic titanium. For example, many of the processes which have been proposed for the production of metallic titanium are based upon a reduction of titanium tetrahalide, such as titanium tetrachloride, with a reducing metal such as sodium, magnesium, etc. In all of such processes, the metallic titanium is formed in the presence of a by-product halide salt of the reducing metal, so that there is a problem of separating the product metal from the by-product salt. At the present time this separation is generally carried out by evaporating the salt from the metal in a high temperature vacuum operation—which is, at best, a very expensive operation.

Since the by-product salts formed in the reduction of titanium tetrahalide with a reducing metal are generally relatively water-soluble, it might appear at first glance that a simple and expedient way to separate said salts from the metallic titanium would be merely to leach the mixture of metal and salts with water to dissolve the salts and leave the metal. As a practical matter, however, the reaction mixture resulting from such a reduction of titanium tetrahalide always contains an appreciable proportion of either or both of (1) unreacted reducing metal or (2) unreacted tetrahalide or partially reduced lower halides. Any unreacted reducing metal in the reduction products will react very rapidly with the water used in leaching and will form a basic solution which will then react with any titanium halides present to form water-insoluble oxygen containing titanium compounds which will contaminate the metallic titanium. Even in the absence of excess reducing metal the titanium halides will hydrolyze in neutral water solutions to form the insoluble oxides or oxychlorides of titanium. Consequently, neutral water solutions are not satisfactory for leaching the salts from mixtures resulting from the commercial reduction of titanium halides with reducing metals.

The aforementioned difficulties resulting from the use of neutral or alkaline leaching solutions can be avoided by utilizing acidic leaching solutions. Any base formed by reaction of excess reducing metal is quickly neutralized by the acid in the solution—and in acidic media any titanium halide will dissolve (rather than hydrolyze to form insoluble oxygen-containing products). While the use of acidic leaching solutions overcomes the difficulties resulting from the use of neutral or basic leaching solutions, it has not heretofore been practical to use acidic solutions because of the high degree of attack by acids upon metallic titanium. This attack is particularly rapid because the metal is generally in a rather finely divided powdered or granular form having a large ratio of surface to volume, so that rather high proportions of the metallic titanium are dissolved in the acidic leaching solution and lost during the leaching process. Thus, the leaching of titanium and salt mixtures with acidic solutions could not be practically useful unless some method were found to reduce the attack by acids upon metallic titanium. It is a preferred object of the present invention to provide such a method.

It has now been found that the use of an organic nitro compound as an inhibitor of acid attack upon metallic titanium is a particularly effective means of reducing said attack. It has been further found that, unlike some inhibitors which have been suggested for use with metallic titanium, the inhibitors of the present invention are particularly effective in the presence of inorganic salts, such as sodium or magnesium chlorides. As a result thereof, it has further been found that aqueous acid solutions containing minor amounts of one or more of said organic nitro compounds are outstandingly effective for leaching inorganic salt by-products from mixtures of said salts with metallic titanium.

The nitro-substituted organic compounds which are useful according to the present invention can be either nitro-substituted cyclic compounds (heterocyclic or carbocyclic) or nitro-substituted aliphatic compounds. The carbocyclic compounds can be either alicyclic or aromatic. The aliphatic and alicyclic compounds can be either saturated or unsaturated.

A preferred class of nitro-substituted compounds of the present invention is the class of nitro-substituted aromatics, and particularly monocyclic aromatics, such as nitrobenzene. Other examples of members of this preferred class of nitro compounds are the nitro-substituted alkylbenzenes, such as the nitrotoluenes, nitroxylenes, nitromesitylenes, nitroethylbenzenes, nitrocumenes, nitrocymenes, nitrostyrenes, etc., in which the nitro group is attached to a carbon atom of the aromatic ring. Other aromatic hydrocarbons, the nitro derivatives of which are suitable for use as inhibitors according to the present invention are the various polycyclic aromatics, fused-ring or otherwise, such as naphthalene, diphenyl, etc.

Examples of suitable non-aromatic carbocyclic nitro-substituted organic compounds are nitrocyclohexane, nitrocyclopentane, 1-nitrocyclopentadiene, and the various hydrocarbyl (especially alkyl) substituted derivatives thereof.

Examples of suitable nitro-substituted heterocyclic organic compounds are the various nitrofurans, nitrothiophenes, nitropyrans, and the like.

Suitable nitro-substituted aliphatic organic compounds are the nitroalkanes, e.g., nitromethane, nitroethane, nitro-iso-propane, nitro-tertiary-butane, nitro-n-pentane, and higher homologues, particularly those having fewer than 15 or 20 carbon atoms therein. Nitro-substituted alkenes such as 3-nitro-propene-1 and nitro aliphatics containing aromatic substituents, e.g.,  $\beta$ -nitroethylbenzene, are also suitable.

The present nitro-organic compounds include not only

the aforementioned compounds, or classes thereof, but also such compounds containing one or more additional nitro groups, or one or more other negative polar groups, e.g., halogen (especially chloro), sulfonic acid or metal sulfonate, hydroxyl, aldehyde, carboxyl, oxo, amide, etc., groups or radicals. Examples of such multi-substituted organic compounds are tetranitromethane, nitrochlorobenzenes, nitroform, nitrobenzyl chloride, nitrobenzene sulfonic acid, sodium nitrobenzene sulfonate, nitroethanol, nitropentane-diol, nitrophenol, nitrobenzyl alcohol, nitronaphthal, nitrobenzaldehyde, nitroacetic acid, nitrobenzoic acid, nitrocinnamic acid, nitrobenzamide, nitroacetophenone, nitroanisol, nitrophenetole, nitrobenzal chloride, nitro phthalic acid or salts or esters thereof, nitroresorcinol, nitrochlorophenol, nitro salicylic acid or salts thereof, nitrophenol sulfonic acid, nitrobenzoyl chloride, and others.

The concentrations of the present inhibitors to be used in any particular application will depend somewhat upon factors such as temperature, acid concentrations, degree of required inhibition, and the presence and concentration of foreign materials such as inorganic salts, etc., but will, in general, range from about 0.01 weight percent to about 10 weight percent, and preferably from about 0.05 weight percent to about 5 weight percent, based upon the amount of acid (or solution thereof) to be inhibited.

As indicated above, the present inhibitors are useful in inhibiting acid corrosion of metallic titanium under numerous circumstances, but are particularly useful in making up aqueous acid leaching solutions for removing inorganic salts, especially halides, e.g., chlorides, from mixtures of such salts with powdered or granular metallic titanium. These acid leaching solutions generally comprise from about 1 to about 25 weight percent, and preferably from about 3 to about 10 weight percent, of

since, as will be seen from the examples which follow hereinbelow, the inhibitors are also effective at higher temperatures and, of course, can be utilized at lower temperatures as well.

5 The time required to leach the salts from the metallic titanium may run anywhere from a few minutes to several hours, depending upon the proportion and type of salt to be leached, concentration of acid in the leaching solution, temperature of leaching operation, physical and chemical states of the salt and metal, the contacting efficiency of the solution with the solids, etc.

10 The following results are presented as illustrative of the highly effective nature of the nitro-organic inhibitors of the present invention, in reducing acid attack upon metallic titanium.

#### EXAMPLE

Numerous nitro-organic compounds were tested for their ability to inhibit acid corrosion upon metallic titanium. In making these tests a weighed sample of powdered (20-60 mesh) metallic titanium was placed in 100 cc. of a water solution of hydrochloric acid, to which solution there was added to a measured amount of a nitro-organic inhibitor. In some cases one gram of sodium chloride was also added in order to determine the effect of the inhibitor in the presence of an inorganic salt. The metal was kept in contact with the acid for a specified length of time, while maintaining the acid at a substantially constant temperature. Any appreciable attack by the acid upon the metallic titanium resulted in the formation of a deep violet color in the solution (formation of titanium trichloride by reaction of hydrochloric acid with titanium). The degree of acid attack was determined by measuring the loss in weight of the titanium sample. The results of these tests are summarized in the following table.

Table

| Inhibitor            |                          | Acid,<br>Wt.<br>Percent | NaCl | Time,<br>Hrs. | Temp.,<br>°C. | Percent<br>Ti, Wt.<br>Loss | Remarks                            |
|----------------------|--------------------------|-------------------------|------|---------------|---------------|----------------------------|------------------------------------|
| Species              | Conc.,<br>Wt.<br>Percent |                         |      |               |               |                            |                                    |
| None                 |                          | 14                      | No   | 1             | 70            | 13.2                       | Solution turned deep violet color. |
| Do                   | 5                        | Yes                     | 18½  | 30            | 5.6           | Do.                        |                                    |
| Do                   | 5                        | Yes                     | 24   | 30            | 5.2           | Do.                        |                                    |
| Nitric acid          | 0.1                      | 14                      | No   | 1             | 70            | 0.4                        | Solution remained colorless.       |
| Do                   | 0.1                      | 14                      | Yes  | 1             | 70            | 16.3                       | Solution turned deep violet.       |
| Nitrobenzene         | 0.5                      | 14                      | No   | 1             | 70            | 0.5                        | Solution remained colorless.       |
| Do                   | 0.5                      | 14                      | Yes  | 1             | 70            | 0.4                        | Do.                                |
| Do                   | 0.2                      | 14                      | Yes  | 1             | 70            | 0.6                        | Do.                                |
| o-Nitrotoluene       | 0.5                      | 5                       | No   | 16            | 30            | 0.2                        | Do.                                |
| Do                   | 0.5                      | 5                       | Yes  | 16            | 30            | ( <sup>1</sup> )           | Do.                                |
| 1-Nitro-n-butane     | 0.5                      | 5                       | No   | 16            | 30            | 0.3                        | Do.                                |
| Do                   | 0.5                      | 5                       | Yes  | 16            | 30            | 0.4                        | Do.                                |
| o-Nitrochlorobenzene | 0.5                      | 5                       | Yes  | 24            | 30            | 0.2                        | Do.                                |
| p-Nitrophenol        | 0.5                      | 5                       | Yes  | 24            | 30            | 0.3                        | Do.                                |
| o-Nitrobiphenyl      | 0.5                      | 5                       | Yes  | 24            | 30            | 0.2                        | Do.                                |

<sup>1</sup> Sample lost during filtration prior to final weighing.

an acid in a water solution. It is, of course, readily apparent that any one of numerous acids would be suitable for this use, since the primary purpose of the acid is merely to supply hydrogen ions to the solution. However, the mineral acids, and particularly those such as hydrochloric and sulfuric acids, are especially suitable because they are substantially completely dissociated in water solutions and are inexpensive and readily available. To these aqueous acid leaching solutions is added one or more of the inhibitors of the present invention in amounts within the range of concentrations indicated above. For a mineral acid solution of from about 3 to 10 weight percent a particularly suitable amount is between 0.1 weight percent and about 2 weight percent, based upon the weight of aqueous acid solution.

Leaching operations carried out with the inhibited leaching solutions of the present invention will generally be carried out at room temperature or thereabouts. This temperature, however, is largely a matter of convenience

I claim:

1. A method of inhibiting corrosion of metallic titanium by acids which comprises incorporating into said acids a corrosion-inhibiting concentration of a nitro-substituted organic compound.

60 2. A method for inhibiting corrosion of metallic titanium by acid solutions which comprises incorporating into said solution a corrosion-inhibiting concentration of at least 0.01 weight percent of a nitro-aromatic compound.

3. A method of inhibiting corrosion of metallic titanium by aqueous acid solutions which comprises incorporating into said solution a corrosion-inhibiting concentration between about 0.05 weight percent and about 5 weight percent of a nitro-substituted aromatic hydrocarbon compound.

70 4. A method of inhibiting corrosion of metallic titanium by aqueous acid solutions which comprises incorporating into said solution a corrosion-inhibiting con-

centration between about 0.05 weight percent and about 5 weight percent of nitrobenzene.

5. A method of leaching a water-soluble inorganic salt from a mixture of said salt and metallic titanium, which method comprises contacting said mixture with an acidic solution containing a corrosion-inhibiting concentration of nitrobenzene to dissolve said salt in said solution, and thereafter separating the metallic titanium from said solution.

References Cited in the file of this patent

UNITED STATES PATENTS

2,134,432 Cantrell et al. Oct. 25, 1938  
2,185,238 Whaley Jan. 2, 1940

2,411,593 Routson Nov. 26, 1946  
2,450,861 Robinson Oct. 5, 1948  
2,639,971 Broyles May 26, 1953  
5 2,662,808 Newschwander Dec. 15, 1953  
2,694,001 Hayes et al. Nov. 9, 1954  
2,707,149 McKinley Apr. 26, 1955

OTHER REFERENCES

10 Bockris et al. in "Chemical Abstracts," vol. 43, col. 952(b), 1949.  
Cobb et al., article, "Resistance of Titanium to Sulfuric and Hydrochloric Acids Inhibited by Ferric and Cupric Ions," in "Journal of the Electrochemical Society," January 1952, pp. 13-15.